

1,433,448.

T. S. CURTIS,  
ELECTRIC FURNACE,  
APPLICATION FILED AUG. 7, 1919.

Patented Oct. 24, 1922.

Fig. 1



Fig. 2



Inventor  
Thomas Stanley Curtis

384

Howard E. Barlow  
Attorney

## UNITED STATES PATENT OFFICE.

THOMAS STANLEY CURTIS, OF PROVIDENCE, RHODE ISLAND, ASSIGNOR TO  
UNIVERSAL OPTICAL CORPORATION, OF PROVIDENCE, RHODE ISLAND, A  
CORPORATION OF RHODE ISLAND.

## ELECTRIC FURNACE.

Application filed August 7, 1918. Serial No. 315,972.

*To all whom it may concern:*

Be it known that I, THOMAS STANLEY CURTIS, a citizen of the United States, and resident of the city of Providence, in the 5 county of Providence and State of Rhode Island, have invented certain new and useful Improvements in Electric Furnaces, of which the following is a specification.

This invention relates to a new method 10 and apparatus for treating magnesite and other ores with electrically generated heat for the purpose primarily of producing a highly refractory material.

The object of this invention is to fuse the 15 material into a dense mass or clinker having its maximum gravity or density.

A further object of this invention is the provision of means whereby the heat-conducting electrodes may be gradually separated 20 during the fusing process for the purpose of enlarging the volume through which the current must pass and so fuse the maximum amount of material during each operation.

25 A still further object of the invention is to so deposit the material about the electrodes that that portion adjacent the electrode will be fused and that portion surrounding the fused portion will be calcined or partially 30 burned whereby when cooled the fused portion may be readily removed in one unbroken lump or mass from the calcined portion, and the calcined portion may be positioned about the electrodes to be fused in a subsequent 35 operation.

With these and other objects in view, the invention consists of certain novel features 40 as will be more fully described, and particularly pointed out in the appended claims.

45 In the accompanying drawings:

Figure 1 is a sectional side elevation of a furnace illustrating my improved method of treating ore.

Figure 2 is an end elevation of the device 45 illustrated in Figure 1.

Referring to the drawings, 10 designates 50 a furnace which may be made in any suitable form but preferably in the present case it is made rectangular, the walls of which may be built up of brick or other suitable refractory material, the side walls 9 being preferably arranged so that they may be readily removed after each operation to facilitate the removal of the charge. The end walls 11

of the furnace are preferably provided with 55 a hole 12 in which is slidably mounted horizontally-disposed electrodes 13 whose inner ends when first positioned are adapted to meet in the center of the furnace and whose outer ends 14 are each supported on a carriage 60 15, whereby they may be withdrawn and separated gradually, either intermittently or continuously as desired, during the treating of the charge in the furnace. Each of these carriages is shown as being movably 65 mounted on wheels 16 to roll on rails 17, the latter being graduated so as to indicate the exact distance each electrode has been withdrawn, and a suitable mechanism such as a crank 18 connected by a sprocket 19 to one of 70 the wheel shafts may be provided if desired, to facilitate the movement of the carriage by the operator.

In building up a charge in this furnace to be operated upon by my improved process, I 75 first deposit a layer 20 of raw or untreated ore on the bottom of the furnace, piling the same up to some extent around the side and end walls for the purpose of protecting these walls against the heat, I then position the 80 electrodes 13 so that their ends will abut, and then deposit in the middle of the furnace about the electrodes a quantity of previously calcined ore 21, or ore partially baked and freed from the greater portion of its carbon dioxide by having been subjected to a moderate degree of heat. I then pour in another 85 layer 22 of raw material over and around this middle portion of calcined material.

The electric current is then turned on 90 which passes through the electrodes 13, an arc being established by slightly separating these electrodes which are further separated from time to time as the charge heats up until at the end of several hours the ends of the electrodes may have been withdrawn nearly to the end walls of the furnace thereby enlarging the volume of material through which the current is caused to pass to obtain the maximum amount of fused material in 95 each charge. The current passing through the highly heated core of magnesite causes it to become a conductor of the current when hot, although this magnesite is an insulator when cold.

100 The outer layer or envelope of raw material serves a double purpose; first, it encloses the inner mass of fused material and

prevents the heat from radiating to and destroying the inclosing walls; second, this outer layer absorbs the heat which is conducted to it from the inner mass while fusing, which heat serves to calcine this outer portion and practically free the same from its contained carbon dioxide providing a partially baked material which will serve as a conducting core for the next succeeding charge.

Thus we have effected a thorough fusion of the core by turning it into a resistor, the withdrawing of the electrodes serving merely to set up a condition of conductivity in successive portions of the core; and we have also effected a preliminary heating or calcination of the surrounding layer of ore which has formed a heat-insulating envelope for the highly heated charge and so have utilized the otherwise wasted heat in each fusing operation.

After this process has been continued for a sufficient length of time the current is turned off and the whole allowed to cool. In practice it has heretofore been found an expensive and difficult operation to remove the fused or sintered portion of the charge from the calcined portion as this fused portion has never before been supported by a broken, unfused mass, but with my improved method of building up the furnace charge it is only necessary after scraping away the loose, now calcined outer layer of material, to hook onto this fused portion and lift the same, by means of grappling irons and a crane, in an unbroken mass of substantially egg shape from its bed of disintegrated, unfused material, with practically none of this unfused ore clinging to it. The side walls of the furnace may be removed if desired to further facilitate the removal of the furnace charge.

If this fused lump is now permitted to fall a distance it will be broken up ready for the crusher. The calcined or remaining portion of the ore in the furnace, which formed the original envelope for the fused portion is now removed from the furnace ready to be

placed in another charge about the electrodes to complete its fusing in a subsequent operation.

Magnesite fused by my improved method forms a refractory which has been shrunk and reduced to its maximum density and, therefore, will not further shrink and for this reason it is most valuable for use in the construction of materials designed to withstand a high degree of heat, such for instance as retorts, furnace linings, crucibles, muffles and for numerous other similar purposes.

Having thus described one illustrative embodiment of my invention and the best mode known to me for carrying out my method, I desire it to be understood that although specific terms are employed, they are used in a generic and descriptive sense and not for the purpose of limitation, the scope of the invention being defined and limited only by the terms of the appended claims.

I claim:

1. In a furnace, horizontally disposed electrodes positioned end to end, a carrier for said electrodes whereby they may be separated and a graduated scale by which the relative positions of said carriers may be readily determined.

2. In a furnace, electrodes projecting through the walls into the furnace and positioned to be covered by the charge, a carrier in which the outer portion of said electrodes is mounted whereby said carrier may be moved to withdraw said electrodes through the charge during the fusing operation.

3. In a furnace, horizontally disposed electrodes positioned end to end, each extending through the walls into the furnace, a carrier for supporting the outer end of said electrodes means whereby said carriers may be moved to regulate the position of said electrodes relative to each other and a graduated member by which the relative position of said carriers may be readily determined.

In testimony whereof I affix my signature.

THOMAS STANLEY CURTIS.